

1

3,058,301

## REACTION MOTOR FUELS

Olaf E. Larsen, Bartlesville, Okla., and Eugene D. Guth, Idaho Falls, Idaho, assignors to Phillips Petroleum Company, a corporation of Delaware  
No Drawing. Filed Dec. 24, 1958, Ser. No. 782,977  
20 Claims. (Cl. 60—35.4)

This invention relates to reaction motor fuels. In one aspect this invention relates to reaction motor fuels suitable for use in reaction motors such as rocket motors, ram jet motors, and the like. In another aspect this invention relates to a method of operating a reaction motor using said new reaction motor fuels.

Rocket motors are operated by burning a mixture of fuel and oxidant in a combustion chamber and causing the resulting gases to be expelled through a nozzle at high velocity. Liquid propellants are frequently preferred over solid propellants where it is necessary to vary thrust during flight. Liquid propellants can be classified as bipropellants and as monopropellants and the latter are either a single compound or mixtures of compounds. The principal elements of a rocket motor utilizing a liquid fuel comprise a combustion chamber, exhaust nozzle, an injection system, and propellant control valves. The propellant gases are produced in the combustion chamber at pressures governed by the chemical characteristics of the propellant, its rate of combustion, and the cross-sectional area of the nozzle throat. The gases are ejected into the atmosphere through the nozzle with supersonic velocity. The function of the nozzle is to convert the pressure of the propellant gases into kinetic energy. The reaction of the discharge of the propellant gases constitutes the thrust developed by the rocket motor.

An object of this invention is to provide a new reaction motor fuel. Another object of this invention is to provide a new reaction motor fuel by employing a suitable emulsifying agent to stabilize an emulsion of an amine nitrate, a liquid hydrocarbon fuel, and nitric acid. Another object of this invention is to provide a new reaction motor, fuel which is suitable for use in a reaction motor such as a rocket motor, a ram jet motor, or the like, for developing thrust. Another object of this invention is to provide a method for operating a reaction motor such as a rocket motor, a ram jet motor, using the reaction motor fuels of the invention. Other aspects, objects, and advantages of the invention will be apparent to those skilled in the art in view of this disclosure.

Thus according to the invention there is provided a fuel composition suitable for use in a reaction motor, comprising, as a stable emulsion, a mixture of (1) from 10 to 60 weight percent of a normally liquid hydrocarbon fuel, (2) from 5 to 50 weight percent of a nitric acid oxidizer containing at least about 70 weight percent of  $\text{HNO}_3$ , (3) from 25 to 60 weight percent of an amine nitrate, and (4) from 1 to 20 weight percent of an emulsifying agent which is chemically non-reactive under the conditions of mixing and storage, i.e., until ignition is effected, with said acid and which is capable of stabilizing an emulsion of said components (1), (2), and (3).

Further according to the invention there is provided a method of operating a reaction motor which comprises the steps of injecting into the combustion chamber of said motor one of the fuel compositions of the invention, igniting and burning said fuel composition, and exhausting gaseous products of combustion from said motor.

As indicated above the reaction motor fuel compositions of the invention comprise an emulsified, non-hypergolic mixture of four components. Mutual compatibility of said components is achieved through the effect of the emulsifying agent. The reaction motor fuels of the inven-

2

tion are particularly suitable for use in ram jet engines. They can be formulated so that oxygen from the air is required for complete combustion and such fuels find ready use in a ram jet engine. For example, fuels containing less than the stoichiometric amount of oxidizer, and which thus require oxygen from the air for complete combustion, can be used in a ram jet motor in the initial phase of operation, e.g., until the ram jet has attained a speed at which sufficient air is available for complete combustion. With complete combustion there is an increase in efficiency of operation. It is thus possible to provide a fuel composition containing a higher percentage of fuel component and a lower percentage of oxidizer component which will be more efficient at normal operating speeds of the ram jet.

However, fuel compositions containing a stoichiometric amount of oxidizer, as well as oxidizer-rich fuel compositions, can also be prepared. Said fuel compositions of the invention containing a stoichiometric amount of oxidizer, and said oxidizer-rich fuel compositions, are, as will be recognized by those skilled in the art, monopropellants, and are suitable for use in rocket motors wherein all of the oxygen necessary for combustion must be injected into the combustion chamber. In those fuel compositions of the invention containing a stoichiometric amount of oxidizer, said stoichiometric amount of oxidizer is defined as the amount required to obtain complete combustion to nitrogen, carbon dioxide, and water. In computing said stoichiometric amount of oxidizer consideration is given to the amount of emulsifying agent which is used to emulsify the mixture of amine nitrate, liquid hydrocarbon fuel, and nitric acid oxidizer. Thus, the stoichiometric amount of oxidizer includes the amount necessary to oxidize said emulsifying agent as well as the amount necessary to oxidize the liquid hydrocarbon and the amine nitrate with which the nitric acid is emulsified. A slightly fuel-rich mixture is usually required to give an optimum rocket motor performance.

In the operation of a reaction motor using the fuel compositions of the invention, said fuel composition can be injected into the combustion chamber of said motor in any suitable manner known to those skilled in the art. After injection into said combustion chamber the fuel composition can be ignited by any suitable means such as, for example, by an electric igniter.

Suitable amine nitrates for use in the practice of the invention include those selected from the group consisting of piperidine nitrate, pyridine nitrate, 2-methylpyridine nitrate, and amine nitrates characterized by a formula selected from the group consisting of



55 and



60 wherein:  $n$  is an integer of from 1 to 5; each  $R_1$  and each  $R_2$  is selected from the group consisting of acyclic, alicyclic, and aromatic hydrocarbon radicals containing from 1 to 8 carbon atoms, and hydrogen, at least one  $R_1$  being one of said hydrocarbon radicals; and  $R_3$  is selected from the group consisting of

(a) alkylene, alkenylene, and alkynylene hydrocarbon radicals containing from 2 to 8 carbon atoms wherein the carbon atoms attached to the nitrogen atoms are attached to adjoining carbon atoms by single valence bonds, and

70 (b)  $\{R_4-X\}R_4$ —radicals wherein each  $R_4$  is an alkyl-

ene radical containing from 2 to 4 carbon atoms, and X is selected from the group consisting of oxygen, sulfur, and



radicals wherein R<sub>2</sub> is as defined above, y is an integer of from 1 to 3, and z is an integer of from 1 to 3; the total number of carbon atoms in the molecule does not exceed 40; and the total number of amino nitrogen atoms in the molecule does not exceed 5.

Examples of amine nitrates which can be used in the practice of the invention include, among others, the following:

Methylamine nitrate  
 Dimethylamine nitrate  
 Trimethylamine nitrate  
 Ethylamine nitrate  
 Diethylamine nitrate  
 Triethylamine nitrate  
 Propylamine nitrate  
 Dipropylamine nitrate  
 Tripropylamine nitrate  
 Isopropylamine nitrate  
 Tertiary butylamine nitrate  
 Isobutylamine nitrate  
 Cyclopentylamine nitrate  
 Cyclohexylamine nitrate  
 Cyclooctylamine nitrate  
 Dicyclohexylamine nitrate  
 Tricyclohexylamine nitrate  
 4-cyclohexenylamine nitrate  
 Phenylamine nitrate  
 Diphenylamine nitrate  
 Tri-n-butylamine nitrate  
 N,N-di-n-octyl-p-tolylamine nitrate  
 o-Methylbenzylamine nitrate  
 N,N,N',N'-tetramethylmethylethane-1,2-diamine dinitrate  
 N,N,N',N'-tetraethylmethylethane-1,2-diamine dinitrate  
 N,N,N',N'-tetra-n-octylethane-1,2-diamine dinitrate  
 N,N,N',N'-tetramethylpropane-1,2-diamine dinitrate  
 N,N,N',N'-tetramethylpropane-1,3-diamine dinitrate  
 N,N,N',N'-tetraethylpropane-1,3-diamine dinitrate  
 N,N,N',N'-tetrabutylpropane-1,3-diamine dinitrate  
 N,N,N',N'-tetrahexylpropane-1,3-diamine dinitrate  
 N,N,N',N'-tetramethylbutane-1,4-diamine dinitrate  
 N,N,N',N'-tetracyclohexylbutane-1,4-diamine dinitrate  
 N,N,N',N'-tetraphenylbutane-1,4-diamine dinitrate  
 N,N,N',N'-tetraphenyl-n-3-octene-1,3-diamine dinitrate  
 N,N,N',N'-tetracyclohexylhexane-2,6-diamine dinitrate  
 N,N,N',N'-tetramethyl-2-butene-1,4-diamine dinitrate  
 N,N,N',N'-tetramethyl-2-butyne-1,4-diamine dinitrate  
 N,N,N',N'-tetramethyloctene-4,8-diamine dinitrate  
 N-phenyl-N'-n-octylethane-1,2-diamine dinitrate  
 N,N,N',N'-tetra-n-octyloctane-1,2-diamine dinitrate  
 N,N'-di(2-ethylhexyl)-2-butene-1,4-diamine dinitrate  
 N,N,N',N'-tetraethyl-4-octyne-1,8-diamine dinitrate  
 Bis-(N,N-dimethylaminoethyl)ether dinitrate  
 Bis-(N,N-di-n-octylamino-n-butyl)ether dinitrate  
 N-cyclohexylaminopropyl N-phenylaminopropyl ether dinitrate  
 N-2-ethylphenylaminoethyl amino-n-butyl ether dinitrate  
 Bis(amino-n-butyl)ether dinitrate  
 Bis(N,N-di-2-ethylcyclohexylamino-n-butyl)thioether dinitrate  
 Bis(aminoethyl)thioether dinitrate  
 Bis(N,N-dimethylaminoethyl)thioether dinitrate  
 N,N,N',N'-tetramethyl-1,3-diamine-2-propanol dinitrate  
 N,N,N',N'-tetraethyl-1,9-diamino-5-nonanol dinitrate  
 N,N',N'-tri-2-ethylcyclohexyl-1,4-diamino-2-butanol dinitrate  
 N,N,N',N',N''-pentamethylidiethylenetriamine trinitrate  
 N,N,N''-tricyclohexylidiethylenetriamine dinitrate

N,N,N'-tri-n-octylidiethylenetriamine trinitrate  
 N,N,N',N'',N''-hexamethylpropane-1,2,3-triamine trinitrate  
 N<sub>1</sub>,N<sub>1</sub>,N<sub>2</sub>,N<sub>2</sub>,N<sub>3</sub>,N<sub>3</sub>,N<sub>4</sub>,N<sub>4</sub>,N<sub>5</sub>,N<sub>5</sub>,N<sub>5</sub>-decamethylpentane-1,2,3,4,5-pentane pentanitrate  
 N<sub>1</sub>,N<sub>2</sub>,N<sub>3</sub>,N<sub>4</sub>,N<sub>5</sub>-pentaethyltetraethylenepentamine pentanitrate  
 N-ethyl-2-butynylamine nitrate  
 N-methyl-2-butynylamine nitrate  
 Di(2-butynyl)amine nitrate  
 N-hexyl-2-propynylamine nitrate  
 N-propyl-3-hexynylamine nitrate

The preferred compounds are the nitrates of primary, secondary, and tertiary mono-amines and tertiary diamines. For these preferred compounds the preferred hydrocarbon R<sub>1</sub> groups are alkyl groups having 1 to 6, inclusive, carbon atoms. For the tertiary diamines, the preferred R<sub>2</sub> groups are alkylene groups having 3 to 6 carbon atoms. These preferred compounds generally have a greater stability in the acid solution. Presently more preferred amine nitrates for use in the practice of the invention include the following:

Piperidine nitrate  
 Pyridine nitrate  
 N,N,N',N'-tetramethylmethylethane-1,2-diamine dinitrate  
 N,N,N',N'-tetramethylpropane-1,2-diamine dinitrate  
 N,N,N',N'-tetramethylpropane-1,3-diamine dinitrate  
 N,N,N',N'-tetramethylbutane-1,3-diamine dinitrate  
 Methylamine nitrate  
 Dimethylamine nitrate  
 Triethylamine nitrate  
 Trihexylamine nitrate

Amine nitrates can be prepared by several methods. One method is to react an amine with nitric acid. Another method which can be employed is to form a salt of the amine, such as a hydrochloride or an acetate, and then react said amine salt with nitric acid. It is also known that amine nitrates can be prepared from amines or amine salts by ion exchange processes. For example, a solution of the amine in a suitable solvent can be contacted with an ion exchange resin which has been previously regenerated by washing the resin with a solution containing the desired anion, e.g., with nitric acid solutions. Further details regarding the preparation of amine nitrates are given in Example I below.

Any suitable emulsifying agent which is chemically non-reactive with nitric acid under the conditions of mixing and storage, i.e., until ignition is effected, and which is capable of stabilizing an emulsion of a liquid hydrocarbon, nitric acid, and an amine nitrate, can be used in the practice of the invention. Examples of suitable emulsifying agents which can be used in the preparation of the rocket fuel compositions of the invention include, among others, the following: (A) Derivatives of imidazoline, also called glyoxaldine, having the structure



where R<sub>5</sub> is an alkyl or alkenyl radical containing from 12 to 18 carbon atoms, and R<sub>6</sub> is OH or NH<sub>2</sub>. Examples of R<sub>5</sub> are dodecyl, tetradecyl, hexadecenyl, heptadecyl, octadecyl, 4-propyl-decyl, and heptadecenyl radicals. Specific compounds include: 1-hydroxyethyl-2-heptadecenyl glyoxaldine (Amine 220), 1-aminoethyl-2-heptadecyl glyoxaldine, 1-hydroxyethyl-2-dodecyl glyoxaldine, and 1-hydroxyethyl-2-octadecyl glyoxaldine; (B) sulfated fatty oils, i.e., esters of glycerol and a 6 to 18 carbon atom aliphatic fatty acid which is sulfated so as to contain sulfated groups or sulfonated so as to contain sulfonated groups in the acid chain, such as: trihexyl sulfotricarbonylate (Nekal NS), castor oil sulfonate (Turkey red oil),

sulfonated tallow (Napco 1497B); (C) aliphatic fatty acid amides which contain from 12 to 18 carbon atoms, such as: dodecanamide, stearamide, oleamide, and hexadecanamide; (D) the condensation products of nonyl phenol with from 4 to 8 mols of ethylene oxide such as Igepal CO-430, and representing the condensation product obtained when 4 mols of ethylene oxide are condensed with one mol of nonyl phenol; (E) N-alkyl trimethylenediamines having alkyl groups with from 12 to 18 carbon atoms such as: N-dodecyl trimethylenediamine, N-heptadecyl trimethylenediamine, and N-octadecyl trimethylenediamine; and (F) copolymers formed by copolymerizing a predominantly non-polar alkyl acrylate monomer with an aminoalkyl acrylate monomer which contains a basic nitrogen atom. Particularly suitable copolymers are those formed by copolymerizing, in parts by weight per 100 parts of monomers, from 5 to 50 parts of at least one monomer selected from the group of alkyl acrylate esters having the formula



with from 95 to 50 parts of at least one monomer selected from the group consisting of aminoalkyl acrylates having the formula



wherein each  $\text{R}_7$  is selected from the group consisting of hydrogen, and alkyl radicals containing from 1 to 3 carbon atoms; each  $\text{R}_8$  is an alkyl radical containing from 10 to 18 carbon atoms; each  $\text{R}_9$  is an alkylene radical containing from 1 to 8 carbon atoms; and each  $\text{R}_{10}$  is selected from the group consisting of hydrogen, and alkyl radicals containing from 1 to 18 carbon atoms.

Suitable predominantly non-polar alkyl acrylate monomers for use in the practice of the invention include, among others, those given in Table I below:

| TABLE I                 |  |
|-------------------------|--|
| Alkyl Acrylate Monomers |  |
| Decyl methacrylate      |  |
| Dodecyl acrylate        |  |
| Dodecyl methacrylate    |  |
| Tetradecyl methacrylate |  |
| Tridecyl methacrylate   |  |
| Hexadecyl methacrylate  |  |
| Octadecyl methacrylate  |  |
| Dodecyl ethacrylate     |  |
| Hexadecyl ethacrylate   |  |
| Dodecyl propacrylate    |  |
| Hexadecyl propacrylate  |  |

Aminoalkyl acrylate monomers containing a basic nitrogen atom which are suitable for use in the practice of the invention include, among others, those given in Table II below:

| TABLE II                           |  |
|------------------------------------|--|
| Aminoalkyl acrylates               |  |
| Aminomethyl acrylate               |  |
| Aminomethyl methacrylate           |  |
| Aminopentyl methacrylate           |  |
| Aminopropyl methacrylate           |  |
| Aminopentyl acrylate               |  |
| Aminohexy1 methacrylate            |  |
| Aminoheptyl methacrylate           |  |
| Aminoocetyl methacrylate           |  |
| Aminomethyl ethacrylate            |  |
| Aminomethyl propacrylate           |  |
| Aminohexy1 ethacrylate             |  |
| Aminoocetyl ethacrylate            |  |
| Amino-2-ethylhexyl acrylate        |  |
| Dimethylaminomethyl methacrylate   |  |
| Diethylaminoethyl acrylate         |  |
| Diisopropylaminoethyl methacrylate |  |

|    |                                                  |
|----|--------------------------------------------------|
| 5  | Dihexylaminoethyl methacrylate                   |
| 10 | Di-(2,4,6-triethoxyethyl)aminoethyl methacrylate |
| 15 | Didodecylaminoethyl methacrylate                 |
| 20 | Diocetadecylaminoethyl methacrylate              |
| 25 | Dimethylaminopropyl methacrylate                 |
| 30 | Dimethylaminobutyl acrylate                      |
| 35 | Dimethylaminopentyl methacrylate                 |
| 40 | Dimethylaminoocetyl methacrylate                 |
| 45 | Dihexylaminoocetyl ethacrylate                   |
| 50 | Diocetylaminooctyl methacrylate                  |
| 55 | Dimethylamino-(2-ethylpropyl) acrylate           |

The above-mentioned acrylate monomers can be copolymerized by any method known to those skilled in the art to form the copolymers used in the practice of the invention. Normally these copolymers are prepared by emulsion, bulk, and solution polymerization processes. For example, said monomers can be emulsified in water and a polymerization catalyst such as benzoyl peroxide added thereto. The polymerization can be effected at temperatures in the range of 20 to 150° C. until the desired degree of polymerization has been effected. The resulting copolymer can be recovered from the reaction mixture after coagulation thereof with sodium chloride. Further information regarding the details of said copolymerization can be found in U.S. Patents 2,138,031 and 2,138,763, issued to George D. Graves on November 29, 1938. Said monomers are preferably copolymerized in amounts, in parts by weight per 100 parts of monomers, ranging from 5 to 50 parts of at least one of said alkyl acrylate monomers with from 95 to 50 parts of at least one of said amino alkyl acrylate monomers.

Suitable copolymers prepared from the above-described monomers and which are suitable for use in the practice of the invention include among others the following:

| TABLE III     |                                                             |
|---------------|-------------------------------------------------------------|
| Monomer Ratio | Copolymers                                                  |
| 40            | decyl methacrylate/aminopentyl methacrylate.                |
| 45            | dodecyl methacrylate/aminopentyl acrylate.                  |
| 50            | tridecyl methacrylate/aminooctyl methacrylate.              |
| 55            | hexadecyl methacrylate/aminoethyl ethacrylate.              |
| 60            | dodecyl ethacrylate/amino-2-ethylhexyl acrylate.            |
| 65            | hexadecyl ethacrylate/diocetadecylaminoethyl methacrylate.  |
| 70            | hexadecyl ethacrylate/dioctadecylaminoethyl methacrylate.   |
| 75            | dodecyl propacrylate/dimethylaminopropyl methacrylate.      |
| 80            | hexadecyl propacrylate/dimethylaminoocetyl methacrylate.    |
| 85            | hexadecyl propacrylate/dimethylaminoocetyl methacrylate.    |
| 90            | dodecyl methacrylate/dihexylaminoocetyl methacrylate.       |
| 95            | dodecyl methacrylate/diethylamino-(2-ethylpropyl) acrylate. |
| 100           | dodecyl acrylate/aminooethyl acrylate.                      |
| 105           | hexadecyl methacrylate/aminooethyl methacrylate.            |
| 110           | octadecyl ethacrylate/didodecyl aminoethyl ethacrylate.     |
| 115           | dodecyl methacrylate/diethylaminoethyl methacrylate.        |
| 120           | dodecyl methacrylate/diethylaminoethyl methacrylate.        |

The presently preferred emulsifying agents are the above-described derivatives of imidazoline and the above-described acrylate polymers.

Since water tends to retard combustion, the nitric acid used in a propellant system is preferably substantially free of water. Thus, the presently most preferred oxidizer is anhydrous nitric acid. However, other more dilute nitric acids can be used in the practice of the invention. White fuming nitric acids and red fuming nitric acids of varying concentrations are available commercially, and all are useful in the practice of this invention. White fuming nitric acid usually contains about 90 to 99 weight percent water. Red fuming nitric acid usually contains about 70 to 90 weight percent  $\text{HNO}_3$ , from 2 to 25 weight percent  $\text{NO}_2$ , and up to about 10 weight percent water. Of course, mixtures of the above-described acids can be employed to give an acid having any intermediate composition, and all are useful as oxi-

dizers in the practice of this invention. Thus, it has been found that nitric acids of all types containing at least about 70 weight percent  $\text{HNO}_3$  are useful as oxidizers in the practice of this invention.

The reaction motor fuel compositions of the invention can be prepared by any suitable method which will give a stable emulsion of the components of said composition.

recovered by filtration, washed with cold acetone or ether, and dried in a vacuum desiccator at room temperature. The melting point and stability of the amine nitrate were then determined. None of the amine nitrates which were prepared were found to be shock sensitive to the blow of a hammer. The results of these runs are given below in Table IV.

TABLE IV

| Run No. | Amine Charged                                                                | Mols<br>Nitric<br>Acid<br>Charged | Percent<br>Aqueous<br>Acid (Wt.<br>Percent<br>$\text{HNO}_3$ ) | Mols<br>Amine<br>Charged | Yield of<br>Amine<br>Nitrate,<br>Percent | M.P. of<br>Amine<br>Nitrate,<br>°C. |
|---------|------------------------------------------------------------------------------|-----------------------------------|----------------------------------------------------------------|--------------------------|------------------------------------------|-------------------------------------|
| 1.      | $\text{N},\text{N},\text{N}',\text{N}''$ -tetramethylethane-1,2-diamine      | 0.606                             | 40.5                                                           | 0.275                    | 96.3                                     | 220-221                             |
| 2.      | $\text{N},\text{N},\text{N}',\text{N}''$ -tetramethylpropane-1,2-diamine     | 0.606                             | 33.4                                                           | 0.275                    | 92.3                                     | 177-179                             |
| 3.      | $\text{N},\text{N},\text{N}',\text{N}''$ -tetramethylbutane-1,3-diamine      | 0.606                             | 40.5                                                           | 0.275                    | 95.0                                     | 115-116                             |
| 3a.     | $\text{N},\text{N},\text{N}',\text{N}''$ -tetramethylbutane-1,3-diamine      | 1.19                              | 70.0                                                           | 0.578                    | 97.0                                     | 115-116                             |
| 4.      | $\text{N},\text{N},\text{N}',\text{N}''$ -tetramethyl-2-butyno-1,4-diamine   | 0.6                               | 41.0                                                           | 0.285                    | 96.4                                     | 145-148                             |
| 5.      | $\text{N},\text{N},\text{N}',\text{N}''$ -tetraethylmethane-1,2-diamine      | 0.6                               | 41.0                                                           | 0.285                    | 76.5                                     | 142-143                             |
| 6.      | $\text{N},\text{N},\text{N}',\text{N}''$ -tetramethylbutane-1,4-diamine      | 0.43                              | 70.0                                                           | 0.208                    | 98.7                                     | 173-174                             |
| 7.      | $\text{N},\text{N},\text{N}',\text{N}''$ -tetramethylbutane-1,2-diamine      | 0.40                              | 70.0                                                           | 0.183                    | 94.3                                     | 173-174                             |
| 8.      | Bis( $\text{N},\text{N}$ -diethylaminoethyl)ether                            | 0.51                              | 70.0                                                           | 1 0.25                   | 72.0                                     | 88-93                               |
| 9.      | $\text{N},\text{N},\text{N}',\text{N}''$ -tetramethyl-1,3-diamino-2-propanol | 0.51                              | 70.0                                                           | 0.25                     | 85.2                                     | 120-124                             |
| 10.     | $\text{N},\text{N},\text{N}',\text{N}''$ -tetraethyl-1,3-diamino-2-propanol  | 0.51                              | 70.0                                                           | 0.25                     | 91.2                                     | 113-114                             |
| 11.     | $\text{N},\text{N},\text{N}',\text{N}''$ -pentamethyldiethylene triamine     | 0.70                              | 70.0                                                           | 0.23                     | 80.0                                     | 162-163                             |
| 12.     | $\text{N},\text{N},\text{N}',\text{N}''$ -hexamethylpropane-1,2,3-triamine   | 0.53                              | 70.0                                                           | 0.173                    | 65.3                                     | 104-106                             |
| 13.     | $\text{N},\text{N}',\text{N}''$ -dimethylmethylethane-1,2-diamine            | 0.505                             | 60.0                                                           | 0.5                      | not<br>recorded                          | 125                                 |
| 14.     | $\text{N},\text{N},\text{N}',\text{N}''$ -tetramethyl-2-butene-1,4-diamine   | 0.44                              | 70.0                                                           | 0.21                     | 88.8                                     | 179-180                             |
| 15.     | $\text{N},\text{N},\text{N}',\text{N}''$ -tetraethylpropane-1,3-diamine      | 0.42                              | 70.0                                                           | 0.2                      | 97.0                                     | 157.5-159.5                         |

<sup>1</sup> In this run, the amine was dissolved in an equal volume of acetone.

Herein and in the claims, unless otherwise specified, a stable emulsion is defined as one in which no appreciable phase separation occurs upon quiescent standing for a period of at least eight hours. Emulsion compositions within the scope of the invention can be prepared having an emulsion stability ranging from eight hours to more than seven days.

A presently preferred method of preparation of the fuel compositions of this invention is to (1) add the emulsifying agent to the liquid hydrocarbon fuel to form a first solution, (2) dissolve the amine nitrate in the nitric acid so as to form a second solution, and (3) mix said first solution and said second solution to obtain a stable emulsion. Any suitable means for mixing said two solutions can be employed. Highly satisfactory results and essentially completely stable emulsions of said components have been prepared by employing conventional stirring equipment such as an impeller immersed in the liquid in conventional manner. Essentially completely stable emulsions have been prepared by stirring or shaking the two above-described solutions for as short a time as 30 seconds. It is preferred to mix said solutions under conditions at which the temperature of the resulting mixture does not exceed 15° C. It is also preferred to store the prepared fuel compositions at reduced temperatures, e.g. below about 15° C.

The following examples will serve to further illustrate the invention.

## EXAMPLE I

A number of runs were made in which polyamine compounds were reacted with nitric acid to form the corresponding amine nitrates. These runs were carried out according to the following procedure.

An amount of the pure polyamine compound was charged to a flask, after which an amount of aqueous nitric acid was charged slowly to said flask by means of a dropping funnel. The temperature of the flask contents was maintained within the range of from 0 to 10° C. by means of an ice bath and by adjusting the rate of addition of the nitric acid to keep the temperature of the reaction mass below 10° C. During the addition of the nitric acid, the flask contents were stirred vigorously. After the nitric acid has been charged, the flask contents were stirred for several minutes to insure complete reaction, after which said flask contents were poured into approximately 5 times its volume of chilled acetone (-10 to -25° C.). The amine nitrate precipitated out. This precipitate was

30 A fuel rich ram jet rocket fuel composition (identified as fuel A below) was prepared by mixing 11.3 parts by weight of an emulsifying agent consisting of 1-hydroxyethyl-2-heptadecenyl glyoxalidine (Amine 220) with 9.3 parts by weight of a low volatility isoparaffinic JP-4 hydrocarbon fuel to give a first solution. A second solution was formed by dissolving 49.4 parts by weight of  $\text{N},\text{N},\text{N}',\text{N}''$ -tetramethylbutane-1,3-diamine dinitrate in 30.0 parts by weight of anhydrous white fuming nitric acid. Said second solution was then mixed with said first solution by stirring with a conventional stirrer for about 30-40 seconds. Upon mixing of said solutions an emulsion which was stable for more than 7 days was obtained.

45 A second fuel composition (identified as fuel B below) was prepared by dissolving 49.4 parts by weight of  $\text{N},\text{N},\text{N}',\text{N}''$ -tetramethylbutane-1,3-diamine dinitrate in 30.0 parts by weight of anhydrous white fuming nitric acid. Said second fuel B thus contained the same ratio of amine nitrate and nitric acid as said first fuel A.

50 A third fuel composition (identified as fuel C below) consisting of  $\text{N},\text{N},\text{N}',\text{N}''$ -tetramethylbutane-1,3-diamine dinitrate and anhydrous white fuming nitric acid in stoichiometric proportions was prepared by dissolving 33.8 parts by weight of said amine nitrate in 66.2 parts by weight of said acid.

55 Said three fuel compositions A, B, and C were then tested for burning rate by placing a portion of each in a separate 8 mm. I.D. test tube. The surface of the tube contents was then ignited and the time required to burn a 2" long section of the tube contents in the presence of air at atmospheric pressure was recorded. The burning rate for each fuel composition in inches per second was then calculated. The results of said burning rate tests were as follows:

| Fuel | Composition—Parts by Weight                                                                                           | Burning<br>Rate,<br>Inches per<br>Second |
|------|-----------------------------------------------------------------------------------------------------------------------|------------------------------------------|
|      |                                                                                                                       |                                          |
| 70 A | (49.4 parts amine nitrate<br>30.0 parts anhydrous WFNA<br>9.3 parts hydrocarbon fuel<br>11.3 parts emulsifying agent) | 0.0350                                   |
| B    | (49.4 parts amine nitrate<br>30.0 parts anhydrous WFNA<br>33.8 parts amine nitrate)                                   | 0.0085                                   |
| C    | (66.2 parts anhydrous WFNA<br>33.8 parts amine nitrate)                                                               | 0.0117                                   |

Typical JP-4 jet fuels are set forth in Table V given below. Fuel #2 in said table is the type used in the above examples.

TABLE V  
Typical JP-4 Jet Fuels

|                                  | 1                | 2      |
|----------------------------------|------------------|--------|
| Distillation, ° F.:              |                  |        |
| Initial BP.....                  | 162              | 131    |
| 5% Evaporated.....               | 218              | 186    |
| 10%.....                         | 240              | 224    |
| 20%.....                         | 266              | 282    |
| 30%.....                         | 290              | 322    |
| 40%.....                         | 312              | 349    |
| 50%.....                         | 331              | 367    |
| 60%.....                         | 358              | 383    |
| 70%.....                         | 381              | 400    |
| 80%.....                         | 408              | 428    |
| 90%.....                         | 443              | 475    |
| 95%.....                         | 468              | 518    |
| End point.....                   | 500              | 547    |
| Residue, Vol. Percent.....       | 1.0              | 1.2    |
| Loss, Vol. Percent.....          | 0.0              | 1.0    |
| Existent Gum, Mg./100 ml.....    | 1.7              | -----  |
| Potential Gum, Mg./100 ml.....   | 1.8              | -----  |
| Freezing Point, ° F.....         | -70              | -93    |
| Reid Vapor Pressure, p.s.i.....  | 1.8              | 2.1    |
| Density, Gr./cc. at 20° C.....   | 0.7720           | 0.7385 |
| Sulfur, Total, Wt. Percent.....  | 0.109            | 0.0034 |
| L. Heat of Comb., B.t.u./lb..... | 18,651<br>(est.) | 19,006 |
| Aniline Point, ° F.....          | 128.5            | -----  |
| Aromatics, Vol. Percent.....     | 13.2             | 0.6    |
| Bromine No.....                  | 1.1              | 1.4    |
| Smoke Point, mm.....             | 24.5             | -----  |
| Smoke Volatility Index.....      | 56.8             | -----  |

EXAMPLE III

In the absence of an emulsifying agent a stable emulsion does not result when an amine nitrate, nitric acid, and a normally liquid hydrocarbon are mixed. Three parts by weight of an amine nitrate solution in anhydrous white fuming acid consisting of 33.8 weight percent of N,N,N',N'-tetramethylbutane-1,3-diamine dinitrate in 66.2 weight percent of said acid were mixed with 3.85 parts by weight of JP-4 fuel No. 2 (see Table V) to give a mixture having the following composition:

|                    | Weight percent |
|--------------------|----------------|
| Amine nitrate..... | 14.7           |
| Nitric acid.....   | 29.2           |
| JP-4 fuel.....     | 56.1           |
|                    | 100.0          |

This mixture did not produce a stable emulsion. After mixing, the mixture separated in less than one minute into two distinct layers, i.e., a hydrocarbon layer and an acid layer.

While the JP-4 jet fuels described in Table V above are of the presently preferred liquid hydrocarbon fuels for use in the practice of the invention, it is to be understood that other normally liquid hydrocarbon fuels can be used. Thus, other hydrocarbon jet fuels can also be used. Suitable normally liquid hydrocarbons which can be used in the practice of the invention include paraffin, cycloparaffin, and aromatic hydrocarbons in the C-5 to C-30 range or mixtures thereof. Examples of such hydrocarbon fuels are normal pentane, normal hexane, normal heptane, benzene, kerosene, isooctane, 2,3-dimethylbutane, diisobutylene, cyclohexene, cyclohexane, isodecane, methylcyclohexane, toluene, hexadecane, pentatricontane, gasoline, naphthas, and the like. Hydrocarbons in the C-5 to C-16 range are preferred.

Since variations and modifications of the invention can be made by those skilled in the art without departing from the scope or spirit of said invention, it is to be understood that all matter herein set forth in the above discussion is merely illustrative and does not unduly limit the invention.

We claim:

1. A fuel composition suitable for use in a reaction motor, consisting essentially of, as a stable emulsion, a mixture of (1) from 10 to 60 weight percent of a nor-

mally liquid hydrocarbon fuel, (2) from 5 to 50 weight percent of a nitric acid oxidizer containing at least about 70 weight percent of HNO<sub>3</sub>, (3) from 25 to 60 weight percent of an amine nitrate selected from the group consisting of piperidine nitrate, pyridine nitrate, 2-methylpyridine nitrate, and amine nitrates characterized by a formula selected from the group consisting of



wherein: n is an integer of from 1 to 5; each R<sub>1</sub> and each R<sub>2</sub> is selected from the group consisting of acyclic, alicyclic, and aromatic hydrocarbon radicals containing from 1 to 8 carbon atoms, and hydrogen, at least one R<sub>1</sub> being one of said hydrocarbon radicals; and R<sub>3</sub> is selected from the group consisting of

(a) alkylene, alkenylene, and alkynylene hydrocarbon radicals containing from 2 to 8 carbon atoms wherein the carbon atoms attached to the nitrogen atoms are attached to adjoining carbon atoms by single valence bonds, and

(b) {R<sub>4</sub>-X}<sub>y</sub>R<sub>4</sub>— radicals wherein each R<sub>4</sub> is an alkylene radical containing from 2 to 4 carbon atoms, and X is selected from the group consisting of oxygen, sulfur, and



radicals wherein R<sub>2</sub> is as defined above, y is an integer of from 1 to 3, and z is an integer of from 1 to 3; the total number of carbon atoms in the molecule does not exceed 40; and the total number of amino nitrogen atoms in the molecule does not exceed 5, and (4) from 1 to 20 weight percent of an emulsifying agent which is chemically non-reactive with said acid under the conditions of mixing and storage and which is capable of stabilizing an emulsion of said components (1), (2), and (3).

2. The composition of claim 1 wherein said amine nitrate is N,N,N',N'-tetramethylbutane-1,3-diamine dinitrate.

3. The composition of claim 1 wherein said amine nitrate is N,N,N',N'-tetramethylbutane-1,4-diamine dinitrate.

4. The composition of claim 1 wherein said amine nitrate is N,N,N',N'-tetramethylbutane-1,2-diamine dinitrate.

5. The composition of claim 1 wherein said amine nitrate is N,N'-dimethylethane-1,2-diamine dinitrate.

6. The composition of claim 1 wherein said amine nitrate is diisopropyl amine nitrate.

7. The composition of claim 1 wherein said emulsifying agent is 1-hydroxyethyl-2-heptadecenyl glyoxalidine.

8. The composition of claim 1 wherein said emulsifying agent is an 80:20 dodecyl methacrylate/diethylaminoethyl methacrylate copolymer.

9. The composition of claim 1 wherein said amine nitrate is N,N,N',N'-tetramethylbutane-1,3-diamine dinitrate and said emulsifying agent is 1-hydroxyethyl-2-heptadecenyl glyoxalidine.

10. The composition of claim 1 wherein said mixture consists essentially of:

49.4 weight percent of N,N,N',N'-tetramethylbutane-1,3-diamine dinitrate;

30.0 weight percent of anhydrous nitric acid;

9.3 weight percent of a low volatility isoparaffinic JP-4 liquid hydrocarbon fuel; and

11.3 weight percent of 1-hydroxyethyl-2-heptadecenyl glyoxalidine.

11. In the method for the development of thrust by the combustion of a fuel in the combustion chamber of a reaction motor, the steps comprising: injecting into said combustion chamber as said fuel component a stable emul-

sion consisting essentially of a mixture of (1) from 10 to 60 weight percent of a normally liquid hydrocarbon fuel, (2) from 5 to 50 weight percent of a nitric acid oxidizer containing at least about 70 weight percent of  $\text{HNO}_3$ , (3) from 25 to 60 weight percent of an amine nitrate selected from the group consisting of piperidine nitrate, pyridine nitrate, 2-methylpyridine nitrate, and amine nitrates characterized by a formula selected from the group consisting of



wherein:  $n$  is an integer of from 1 to 5; each  $\text{R}_1$  and each  $\text{R}_2$  is selected from the group consisting of acyclic, alicyclic, and aromatic hydrocarbon radicals containing from 1 to 8 carbon atoms, and hydrogen, at least one  $\text{R}_1$  being one of said hydrocarbon radicals; and  $\text{R}_3$  is selected from the group consisting of

(a) alkylene, alkenylene, and alkynylene hydrocarbon radicals containing from 2 to 8 carbon atoms wherein the carbon atoms attached to the nitrogen atoms are attached to adjoining carbon atoms by single valence bonds, and

(b)  $\text{fR}_4-\text{X}\text{f}_y\text{R}_4-$  radicals wherein each  $\text{R}_4$  is an alkylene radical containing from 2 to 4 carbon atoms, and  $\text{X}$  is selected from the group consisting of oxygen, sulfur, and



radicals wherein  $\text{R}_2$  is as defined above,  $y$  is an integer of from 1 to 3, and  $z$  is an integer of from 1 to 3; the total number of carbon atoms in the molecule does not exceed 40; and the total number of amino nitrogen atoms in the molecule does not exceed 5, and (4) from 1 to 20 weight percent of an emulsifying agent which is chemically non-reactive with said acid under the conditions of mixing and storage and which is capable of stabilizing an emulsion of said components (1), (2), and (3); igniting and burning said mixture; and exhausting gaseous products of combustion from said motor.

12. The method of claim 11 wherein said amine nitrate is  $\text{N},\text{N},\text{N}',\text{N}'$ -tetramethylbutane-1,3-diamine dinitrate.

13. The method of claim 11 wherein said amine nitrate is  $\text{N},\text{N},\text{N}',\text{N}'$ -tetramethylbutane-1,4-diamine dinitrate.

14. The method of claim 11 wherein said amine nitrate is  $\text{N},\text{N},\text{N}',\text{N}'$ -tetramethylbutane-1,2-diamine dinitrate.

15. The method of claim 11 wherein said amine nitrate is  $\text{N},\text{N}'$ -dimethylmethane-1,2-diamine dinitrate.

16. The method of claim 11 wherein said amine nitrate is diisopropyl amino nitrate.

17. The method of claim 11 wherein said emulsifying agent is 1-hydroxyethyl-2-heptadecenyl glyoxalidine.

18. The method of claim 11 wherein said emulsifying agent is an 80:20 dodecyl methacrylate/diethylaminoethyl methacrylate copolymer.

19. The method of claim 11 wherein said amine nitrate is  $\text{N},\text{N},\text{N}',\text{N}'$ -tetramethylbutane-1,3-diamine dinitrate and said emulsifying agent is 1-hydroxyethyl-2-heptadecenyl glyoxalidine.

20. A fuel composition suitable for use in a reaction motor, consisting essentially of, as a stable emulsion, a mixture of (1) from 10 to 60 weight percent of a normally liquid hydrocarbon fuel, (2) from 5 to 50 weight percent of a nitric acid oxidizer containing at least about 70 weight percent of  $\text{HNO}_3$ , (3) from 25 to 60 weight percent of an amine nitrate selected from the group consisting of piperidine nitrate, pyridine nitrate, 2-methyl-pyri-

75

dine nitrate, and amine nitrates characterized by a formula selected from the group consisting of



wherein:  $n$  is an integer of from 1 to 5; each  $\text{R}_1$  and each  $\text{R}_2$  is selected from the group consisting of acyclic, alicyclic, and aromatic hydrocarbon radicals containing from 1 to 8 carbon atoms, and hydrogen, at least one  $\text{R}_1$  being one of said hydrocarbon radicals; and  $\text{R}_3$  is selected from the group consisting of

(a) alkylene, alkenylene, and alkynylene hydrocarbon radicals containing from 2 to 8 carbon atoms wherein the carbon atoms attached to the nitrogen atoms are attached to adjoining carbon atoms by single valence bonds, and

(b)  $\text{fR}_4-\text{X}\text{f}_y\text{R}_4-$  radicals wherein each  $\text{R}_4$  is an alkylene radical containing from 2 to 4 carbon atoms, and  $\text{X}$  is selected from the group consisting of oxygen, sulfur, and



radicals wherein  $\text{R}_2$  is as defined above,  $y$  is an integer of from 1 to 3, and  $z$  is an integer of from 1 to 3;

the total number of carbon atoms in the molecule does not exceed 40, and the total number of amino nitrogen atoms in the molecule does not exceed 5, and (4) from 1 to 20 weight percent of an emulsifying agent which is chemically non-reactive with said acid under the conditions of mixing and storage and which is capable of stabilizing an emulsion of said components (1), (2), and (3); said emulsifying agent being selected from the group consisting of: derivatives of glyoxalidine having the formula



wherein  $\text{R}_5$  is selected from the group consisting of alkyl and alkenyl radicals containing from 12 to 18 carbon atoms, and  $\text{R}_6$  is selected from the group consisting of  $\text{OH}$  and  $\text{NH}_2$  radicals; sulfated esters of glycerol and an aliphatic fatty acid containing from 6 to 18 carbon atoms; sulfonated esters of glycerol and an aliphatic fatty acid containing from 12 to 18 carbon atoms; aliphatic fatty acid amides containing from 12 to 18 carbon atoms; condensation products of nonyl phenol with from 4 to 8 mols of ethylene oxide;  $\text{N}$ -alkyl trimethylenediamines wherein the alkyl group contains from 12 to 18 carbon atoms; and copolymers formed by copolymerizing, in parts by weight per 100 parts of monomers, from 5 to 50 parts of at least one monomer selected from the group consisting of alkyl acrylate esters having the formula



with from 95 to 50 parts of at least one monomer selected from the group consisting of aminoalkyl acrylates having the formula



wherein: each  $\text{R}_7$  is selected from the group consisting of hydrogen, and alkyl radicals containing from 1 to 3 carbon atoms; each  $\text{R}_8$  is an alkyl radical containing from 10 to 18 carbon atoms; each  $\text{R}_9$  is an alkylene radical containing from 1 to 8 carbon atoms; and each  $\text{R}_{10}$  is selected from the group consisting of hydrogen,

and alkyl radicals containing from 1 to 18 carbon atoms.

2,645,079  
2,739,981

Doumani et al. \_\_\_\_\_ July 14, 1953  
Szabo et al. \_\_\_\_\_ Mar. 27, 1956

References Cited in the file of this patent

UNITED STATES PATENTS

2,542,193 Hannum \_\_\_\_\_ Feb. 20, 1951  
2,573,471 Malina et al. \_\_\_\_\_ Oct. 30, 1951  
2,636,342 Cade \_\_\_\_\_ Apr. 28, 1953  
2,637,161 Tschinkel \_\_\_\_\_ May 5, 1953

5

133,508

FOREIGN PATENTS

Australia \_\_\_\_\_ July 14, 1949

OTHER REFERENCES

Cottrell et al.: "Journal Chemical Society" (1951),  
pp. 1798-1800.